

## 1

2,915,394

## STABILIZER FOR SINGLE POWDER PHOTOGRAPHIC DEVELOPER

Jerry S. Krizka, Binghamton, N.Y., assignor to General Aniline & Film Corporation, New York, N.Y., a corporation of Delaware

No Drawing. Application December 29, 1955  
Serial No. 556,042

2 Claims. (Cl. 96—66)

The present invention relates to single powder photographic developers, and more particularly to compositions containing organic stabilizers for effectively preventing reaction between the developing agent and the alkaline ingredients of such compositions.

The advantages of single powder photographic developers are readily recognized in that such powders may be blended in one operation and packaged in a simple, single-component container. Such powders contain the usual components for photographic developers such as the developing agents, anti-oxidant or preservative, alkali energizer and an anti-fogging agent. It has been found, however, that when these components are blended in the form of a dry powder there is a marked tendency for the organic developing agent to react with the alkali, causing deterioration of the photographic properties of the composition. It is, therefore, necessary to incorporate in the powder a substance which will preclude such reaction and operate to stabilize the developer.

Recognition of this fact has led the art to select as stabilizers, such substances as benzoic, maleic, boric and phthalic anhydrides and metaboric, salicylic and phthalic acids. Optimum results, however, are not secured by utilization of any of these components. Thus, many are only moderately effective and display properties which lead to additional problems. For example, they cannot be employed with any degree of success where anhydrous sodium carbonate is employed as the alkali. Similarly, they are of little use should it be desired to employ benzotriazole as a blue-black toner or as a restrainer. Again, they dissolve relatively slowly in water, thereby greatly prolonging the mixing operation designed to produce the active developing solutions. Finally, these acidic substances have a tendency to react with sulfite and carbonate, thereby forming gases which may build up objectionable pressures in hermetically sealed containers.

It has now been discovered that the disadvantages of the previously suggested stabilizers may be overcome while obtaining single powder developers, readily soluble in water with little tendency to gas formation during storage, by employing anhydrous oxalic acid as the stabilizer. Single powder developers containing anhydrous oxalic acid as a stabilizer constitute the purposes and objects of the present invention.

The single powder developers contemplated herein contain the usual developer components, such as the developing agent, i.e., metol, phenidone, hydroquinone, p-aminophenol, hydrochloride, pyrogallol and the like; a preservative or anti-oxidant such as an alkali metal sulfite, i.e., potassium sulfite, potassium metabisulfite and the like; an alkali energizer such as sodium carbonate, borax or the like; and an anti-fogging agent such as potassium bromide and the like.

The oxalic acid is added to the composition in an amount ranging from .5 to 5% by weight of the dry ingredients of the composition. Best results are procured by first mixing the alkaline ingredients with the oxalic acid and then adding the remaining ingredients and blending the whole to a uniform mixture.

As previously indicated, the oxalic acid tolerates the

## 2

presence of benzotriazole and, hence, this component may be used in the compositions hereof, either as a restrainer or to produce blue-black tones. It is also recommended that a sequestering agent be added to take care of salts present in hard water and, to this end, ethylene diamine tetra acetic acid may be effectively employed.

The following examples will serve to illustrate the invention, but it is to be understood that the invention is not restricted thereto. The components of the various examples may be packaged as single powder mixtures for dissolution in one liter of water to prepare the developer solution.

## Example I

|                                       | Grams |
|---------------------------------------|-------|
| 15 Ethylene diamine tetra acetic acid | 0.8   |
| Borax                                 | 4.0   |
| Oxalic acid, anhydrous                | 0.6   |
| Sodium sulfite                        | 80.0  |
| Metol                                 | 1.5   |
| 20 Hydroquinone                       | 3.0   |
| Potassium bromide                     | 0.5   |

## Example II

|                                       | Grams |
|---------------------------------------|-------|
| 25 Ethylene diamine tetra acetic acid | 0.5   |
| Sodium sulfite                        | 44.0  |
| Oxalic acid, anhydrous                | 0.6   |
| Diamino phenol hydrochloride          | 6.6   |
| Potassium bromide                     | 0.55  |

## Example III

|                                       | Grams |
|---------------------------------------|-------|
| 35 Ethylene diamine tetra acetic acid | 0.8   |
| Sodium carbonate, monohydrate         | 25.0  |
| Oxalic acid, anhydrous                | 1.0   |
| Potassium metabisulfite               | 2.5   |
| Sodium sulfite                        | 13.0  |
| Metol                                 | 1.3   |
| Hydroquinone                          | 3.7   |
| Benzotriazole                         | 0.006 |
| 40 Potassium bromide                  | 0.3   |

## Example IV

|                                       | Grams |
|---------------------------------------|-------|
| 45 Ethylene diamine tetra acetic acid | 0.8   |
| Sodium carbonate, monohydrate         | 27.0  |
| Oxalic acid, anhydrous                | 1.0   |
| Potassium metabisulfite               | 2.5   |
| Sodium sulfite                        | 10.0  |
| Phenidone                             | 0.10  |
| Hydroquinone                          | 6.0   |
| 50 Benzotriazole                      | 0.006 |
| Potassium bromide                     | 0.3   |

## Example V

|                                      | Grams |
|--------------------------------------|-------|
| 55 Ethylenediamine tetra acetic acid | 1.0   |
| Sodium carbonate, anhydrous          | 23.0  |
| Oxalic acid, anhydrous               | 1.0   |
| Potassium metabisulfite              | 2.5   |
| Sodium sulfite                       | 10.0  |
| 60 Phenidone                         | 0.10  |
| Hydroquinone                         | 6.0   |
| Benzotriazole                        | 0.006 |
| Potassium bromide                    | 0.3   |

## Example VI

|                                       | Grams |
|---------------------------------------|-------|
| 65 Ethylene diamine tetra acetic acid | 1.0   |
| Sodium carbonate, monohydrate         | 75.0  |
| Oxalic acid, anhydrous                | 3.0   |
| Sodium sulfite                        | 55.0  |
| 70 Potassium bromide                  | 10.0  |
| Hydroquinone                          | 35.0  |

Developers as constituted according to the examples, after storage for prolonged periods at 120° F., showed no significant decomposition and evidenced no gas formation when placed in hermetically sealed cans. However, omission of the oxalic acid caused the mixtures of the examples to become badly discolored after one day's storage with a marked deterioration in their photographic activity.

All of the compositions of the examples dissolved readily in water to form developing solutions photographically equal to those freshly prepared from the individual chemical constituents.

I claim:

1. A stabilized single powder developing composition consisting essentially of an organic silver halide developer selected from the group consisting of methyl-p-amino phenol sulfate, 1-phenyl-3-pyrazolidone, hydroquinone, p-aminophenol hydrochloride, pyrogallol and mixtures thereof, an alkali selected from the group consisting of alkali carbonates, sulfites, borates and mixtures thereof, a stabilizing agent consisting essentially of anhydrous oxalic acid, an antifogging agent and ethylene diamine tetracetic acid.
2. A stabilized single powder developing composition

5  
10  
15

consisting essentially of an organic silver halide developer selected from the group consisting of methyl-p-amino phenol sulfate, 1-phenyl-3-pyrazolidone, hydroquinone, p-aminophenol hydrochloride, pyrogallol and mixture thereof, an alkali selected from the group consisting of alkali carbonates, sulfites, borates and mixtures thereof, ethylene diamine tetra acetic acid, benzotriazole, an antifoggant and a stabilizing agent consisting essentially of anhydrous oxalic acid.

References Cited in the file of this patent

UNITED STATES PATENTS

- |           |                    |               |
|-----------|--------------------|---------------|
| 2,162,765 | Tarnoff -----      | June 20, 1939 |
| 2,649,376 | Rasch et al. ----- | Aug. 18, 1953 |

FOREIGN PATENTS

- |                   |                     |              |
|-------------------|---------------------|--------------|
| 16,537<br>of 1888 | Great Britain ----- | Aug. 3, 1889 |
| 725,892           | Great Britain ----- | Mar. 9, 1955 |

OTHER REFERENCES

Chemistry of Carbon Compounds, Rodd, vol. I, part B (1952), page 955. (Copy in Div. 38.)